

(No Model.)

EUGEN BARON RITTER & CHARLES KELLNER.

PROCESS OF MANUFACTURING CELLULOSE OR PAPER PULP FROM  
WOOD FIBER.

No. 329,215.

Patented Oct. 27, 1885.



WITNESSES:

*C. Williamson.*

*M. L. Gollamer.*

*Eugen, Baron Ritter  
Charles Kellner*

INVENTOR<sup>S</sup>

BY *Conrad F. Ritter*  
ATTORNEYS

# UNITED STATES PATENT OFFICE.

EUGEN BARON RITTER AND CHARLES KELLNER, OF PODGORA, NEAR GOERZ,  
AUSTRIA-HUNGARY, ASSIGNEES TO WILLIAM A. RUSSELL, TRUSTEE, OF  
LAWRENCE, MASSACHUSETTS.

## PROCESS OF MANUFACTURING CELLULOSE OR PAPER-PULP FROM WOOD FIBER.

SPECIFICATION forming part of Letters Patent No. 329,215, dated October 27, 1885.

Application filed January 13, 1885. Serial No. 152,755. (No specimens.) Patented in Austria-Hungary August 2, 1883, No. 20,024 and No. 31,730; in France September 27, 1883, No. 157,754; in Belgium September 29, 1883, No. 62,746, and in Italy January 22, 1884, No. 16,316.

*To all whom it may concern:*

Be it known that we, EUGEN BARON RITTER and CHARLES KELLNER, subjects of the Emperor of Austria-Hungary, residing at 5 Podgora, near Goerz, Austria-Hungary, have invented certain new and useful Processes of Manufacturing Cellulose or Paper-Pulp from Wood Fiber, (the said invention having been patented to us in Italy January 22, 1884, No. 16,316; in France September 27, 1883, No. 157,754; in Belgium September 29, 1883, No. 62,746, and in Austria-Hungary August 2, 1883, No. 20,024 and No. 31,730,) and we do hereby declare the following to be a full, clear, and exact description of the invention, reference being had to the accompanying drawing, which forms a part of this specification.

This invention has relation to the manufacture of cellulose or paper-pulp from woody fiber by the action of sulphurous-acid solution or its equivalent upon the fiber; and the invention consists in a novel process whereby the disaggregation and bleaching of the fibrous material constitutes a single continuous operation.

The details of our process admit of several variations without departure from the spirit of the invention. Thus, for instance, according to one method of carrying our process into effect, woods from which white and strong cellulose is to be manufactured are soaked in vertical stationary boilers containing the disintegrating-solution, and prior to each heating sulphurous acid is forced in until a pressure of at least two atmospheres has been created, when either pure steam or steam mixed with sulphurous acid is admitted and maintained for a long time at a temperature exceeding the boiling-point of water, to be ultimately brought to a temperature corresponding to a pressure of steam amounting to three to five atmospheres. The process thus conducted is disaggregation in its first stage, and in its second stage also bleaching. The material falls out of the boiler in a white state and without any very hard portions, so that it can be manufactured into paper without having to pass through a

knotting apparatus. The boiling process lasts about fourteen to eighteen hours; but it may be extended to thirty-six hours when it is desired to work with less pressure. If, however, the process is to be shortened without weakening the fiber, the boiling process with change of lyes on the principle of the counter-current is employed.

For the better understanding of the steps involved in the method of carrying out our process last referred to, let it be assumed that two communicating boilers or digesters are employed. These boilers we will designate by the letters A B in the accompanying drawing. It is also to be understood that we have at command a supply of acid or sulphite solution already employed twice, and that the fresh wood in either boiler is to be first subjected to the action of this solution.

Let it be supposed that the continuous process has been carried on for some time, and that at one of its stages boiler A contains wood which has been treated with liquid already employed twice, and that boiler B has been filled with fresh wood. From this point on the process continues as follows: First, the liquid from boiler A—that is to say, the twice-used liquid—is forced into boiler B, while fresh liquid is forced into the boiler A, steam admitted also, and the boiling effected. At the same time boiling is going on in boiler L with the liquid which is now being used for a third time. After this latter boiling is completed the sulphurous acid is blown off with the steam from boiler B into a condensing apparatus, C, and the liquid into a collecting-cistern, D, leaving only the partially-disintegrated wood in boiler B. The liquid from boiler A is now forced into boiler B, and is now liquid which has been used but once. Boiling now again takes place in boiler B. Boiler A is now emptied and filled with fresh wood. At this point the conditions of the process are reversed—that is to say, boiler B contains wood which has been treated with liquid already used twice, while boiler A contains fresh wood. Here the operation com-

mences again and continues as before through the courses as above described, boiler B now taking the place of boiler A, and vice versa.

It will be observed that when but two boilers are employed the liquid is used only three times. If, however, a larger number of boilers are employed, the liquid may be forced from one boiler to another throughout the whole series and used from four to eight times, thus materially shortening the boiling process and creating a product which cannot be produced by any other known process. If, however, it is of little consequence whether the fiber obtained is less strong and white than the product of the above-described operation, the interchange of liquid between several boilers may be omitted and rotary boilers having little circumferential velocity employed.

Where the pulp is to be manufactured from hard wood, the rotary boilers are preferably employed.

We have referred in describing our process to the employment of a sulphurous-acid solution, and in this connection we would have it understood that while we do not limit ourselves to the use of a solution of any specific chemical character, we, however, prefer and recommend the use of the double salt of sulphite of calcium magnesium, the constitution thereof being in the proportions of about three atoms of the acid to one of the base. The method of production is described in the application of even date herewith.

In describing our process involving the interchange of the solution between two boilers, we have referred to the introduction of steam containing much sulphurous acid from one boiler to another. By this means we prevent the evolution of the sulphite of calcium, and are enabled to carry on the continuous operation by causing the steam containing much sulphurous acid to blow off from one boiler into another.

We are aware that in the manufacture of paper-pulp from wood fiber it is not new to subject the wood fiber to the action of sulphurous acid and sulphite solutions in a closed vessel under steam-pressure under such conditions that the wood has been practically disintegrated and rendered suitable for the manufacture of paper; but hitherto, so far as we are aware, the sulphite solutions employed have consisted of sulphurous acid combined with a single base, and the processes have resulted in disintegration only, the bleaching of the fiber being omitted or obtained by a separate and independent operation. We have discovered that by employing a solution consisting of the sulphurous acid combined with a double base in certain proportions, and sub-

jecting the wood to the same according to the conditions specified, we not only disintegrate the wood, but we also bleach the same, both results being accomplished in and by the one continuous operation. Our process in its entirety is further distinguished from the processes hitherto employed in respect to the practice of the method of interchanging the solution from one boiler or digester to another, so as to subject the wood at different stages of treatment to the action of fresh solution, whereby the disintegrating and bleaching is facilitated and the process rendered economical.

Having now described our invention, what we claim, and desire to secure by Letters Patent, is—

1. In the manufacture of cellulose or paper-pulp from wood fiber, the process of disintegrating and bleaching the fiber in one continuous operation, consisting, essentially, in subjecting the fiber to the action of a double salt solution wherein sulphurous acid is combined with a double base in the proportions of about three atoms of the acid to one atom of the base in a closed vessel or boiler to which steam is admitted, substantially as described.

2. In the manufacture of cellulose or paper-pulp from wood fiber by one continuous operation, the process of disintegration and bleaching, which consists in first soaking the wood in a disintegrating-solution in a closed vessel, then, prior to heating, forcing in sulphurous acid until a pressure of at least two atmospheres is created, then forcing in steam, or steam mixed with sulphurous acid, and maintaining the contents of the boiler at a temperature exceeding that of boiling water, and finally bringing the temperature to a point corresponding to a steam-pressure of three to five atmospheres, substantially as described.

3. In the manufacture of cellulose or paper-pulp from wood fiber by the action of sulphite solutions, the method of facilitating the disintegration and bleaching operations, which consists in an alternation of the solution between two or more boilers or digesters containing the fiber under different conditions of treatment, whereby each charge of fresh wood is subjected to the action of a solution already used and next subjected to the action of fresh solution, substantially as described.

In testimony that we claim the foregoing we have hereunto set our hands this 28th day of November, 1884.

EUGEN BARON RITTER.  
CHARLES KELLNER.

Witnesses:

APPAD VON BARBER,  
ALBERT VON BARBER.